# EUROPEAN PATENT SPECIFICATION

(11) **EP 0 660 175 B1**
(45) Date of publication and mention of the grant of the patent: **22.03.2000**
(21) Application number: 94119119.9
(22) Date of filing: 05.12.1994
(51) Int. Cl.: G03C 5/31, G03C 5/30

(54) **Control of replenishment during photographic development**
Steuerung der Nachfüllung und Regenerierung während der photographischen Entwicklung
Contrôle du remplissage pendant le développement photographique

(30) Priority: 22.12.1993 US 168422
(43) Date of publication of application: 28.06.1995
(73) Proprietor: Sterling Diagnostic Imaging, Inc., Glasgow, DE 19702 (US)
(72) Inventor: Wuelfing, Peter, Arden, North Carolina 28704 (US)
(74) Representative: Van Ostaeyen, Marc Albert Jozef

(56) References cited:
- EP-A- 0 573 700
- GB-A- 1 313 796
- US-A- 3 529 529
- US-A- 4 741 991

## Description

### Field of Invention:

This invention is related to chemical processing of photographic film. More specifically this invention is related to improved processing mixtures, and a diagnostic test therefore, which allows for accurate determination of replenishment and which provides a method for diagnosing improper replenishment.

### Background of the Invention:

In the photographic process, an image-wise exposed film must be processed to convert the latent image into a viewable negative of the image. The processing operation requires a development step, wherein the exposed silver halide crystals are reduced to elemental silver, and a fix or bleach step wherein the unexposed silver halide crystals are removed from the film. It is also advantageous to wash the film prior to drying and viewing.

Development is accomplished by the reduction of exposed silver halide to silver metal. When hydroquinone, or an equivalent, is used as the reducing agent the reaction which occurs is represented by Equation 1. The active ingredients, hydroquinone and sodium sulfite, are depleted by the silver reduction reaction. Because of the chemical depletions the effectiveness of the processing solution decreases with use. Also occuring is an increase in the bromide level and a decrease in the pH.

Ascorbic acid based developers are also used for reduction of exposed silver halide during development. Analogous depletion of active ingredients is observed with use.

Methods of replenishing the active ingredients are well known in the art and most modern processors are equipped with tanks of replenishment solution and an automatic replenishment mode based on various criteria as known in the art.

Hydroquinone developers are also susceptible to air oxidation. The chemical reaction associated with air oxidation is provided in Equation 2. Air oxidation of a hydroquinone developer does not effect the bromide level but the pH increases due to liberation of hydroxide ion as the sodium salt.

Evaporation of water is also known to occur. Loss of solvent can alter the concentration of ingredients and the reactivity. Yet another detrimental phenomenon is the physical removal of developer solution by the film.

Under standard operating conditions decreases in developer activity are expected due to the development reaction, oxidation reaction, solvent evaporation and physical removal. All of these detrimental phenomenon occur, albeit at different rates. When a large amount of film is processed the development reaction is dominant and the problems which must be addressed are decreasing active ingredients, increasing bromide and decreasing pH. When a small amount of film is processed, or for periods of inactivity, the oxidation reaction and solvent evaporation are the dominant concerns.

Monitoring the bromide in the developer is advantageous for suggesting hydroquinone depletion as detailed in U.S. Patents 3,529,529 and 3,970,457 yet oxidation is not addressed with this method. In practice these automatic systems are known to fail which is blamed, in part, on the lack of an effective method for standardizing electrodes that are continuously monitored. Monitoring pH is not considered to be effective since competing development and oxidation reactions could balance with no substantial change in pH. Also, most modern developer solutions contain pH buffers which may mask changes. Monitoring both bromide and pH places a burden on the user and is typically neither feasible nor diagnostic.

Specific gravity is another analytical measurement which is often used during the initial makeup of the solutions. The inaccuracy and non-specificity of this method is well known in the art and diagnostic information is rarely obtained.

Further, GB-A-1313796 discloses a method for measurement of halide by titration and of hydroquinone by redox titration employing multiple halide additions.

There has been a long felt need in the art to provide a diagnostic measurement whereby the chemicals and their replenishment can be optimized. Preferred is a single measurement which can provide the diagnostic information.

The prior art also suffers from the lack of diagnostic information provided by the above mentioned measurements. For example, a high bromide ion concentration in the developer would suggest more replenishment chemicals need to be added as described for hydroquinone systems in U.S. Pat. Nos. 3,529,529 and 3,970,457. If oxidation, or evaporation, has occured in the replenishment solution, or if the replenisher is incorrectly prepared the bromide ion concentration alone may provide an inaccurate assessment of developer strength.

The ineffective quantitative means of determining chemical activity has led to the design of indirect methods to determine chemical activity of the developer. The standard method in the art has been to process film and monitor the photographic response as detailed in U.S. Patents 5,063,583; 4,508,686 and 4,365,895. A similar approach has been adopted by the American College of Radiology and is manifested in their recommendations for accreditation under the processing section of their Mammography Accreditation Program. These methods are all predicated on the assumptions that:
a) the film samples are identical and stable with time;
b) exposure and density readings are invariant;
c) the developer used at the start of the test is correct; and
d) changes in chemistry will have a predictable, or noticeable, effect on the film.
In actual practice all of these assumptions may, and do, fail.

The choice of film is also critical as realized in the art. Films which utilize tabular grains are known to exhibit sensitometric properties which vary with bromide level in the developer. Films with more conventional grains are known to be less sensitive to bromide level but sensitometric differences correlate more strongly to processing temperature and other changes in developer. This places a burden on the health care professional since different films could exhibit different properties in the same processor. To adequately use the indirect method a control film would have to be established for all types of films employed.

A particular deficiency of prior art tests is the lack of information on the activity of the replenisher chemicals. The bromide titration, or indirect film methods, only test the activity of the development solutions in the processor at the time of the test. A single test provides no information about the replenishment conditions. To obtain information on replenishment a subsequent test must be done and the data correlated to analyze for trends and/or the replenisher must be checked independently. Furthermore, a film method is intrusive since the test film itself initiates the development reaction and some replenishment occurs to compensate therefor. Immediately after the control film is processed the conditions in the development solution will be different.

An improperly prepared replenisher may take a considerable amount of time (several hours to several days) to displace a sufficient amount of developer to be observed by a film test. Nominal replenishment rates, as expected for moderate film use, are sufficient to replace approximately half of the chemicals in the developer tank with replenisher chemicals in approximately 8-10 hours. The full effect of incorrect replenishment, either rate or composition, may not be noticed until the developer has been replaced by at least one equal volume of replenisher. This creates a lag time between replenisher preparation, or a change in the rate of addition, and the actual sensitometric effect. The lag time can span several days in some instances. Once an actual problem is detected the entire replenisher and developer must be replaced to correct the situation.

It is not uncommon that specific chemical changes combine with film choice to generate a rapidly deteriorating problem. If the film is particularly sensitive to specific changes in chemistry a deterioration in performance may occur from the time the new replenisher is prepared. The deterioration in performance may not be realized for quite some time, particularly when large batches of film are processed. This problem is especially troublesome in cases such as mammographic exams where mobile units acquire the exposed films and return to a central processing center wherein all of the films are processed prior to being observed.

The tardiness of the test is especially critical if recommended procedures are followed in entirety. Corrective action is suggested only after three consecutive test are observed to generate a trend in any direction away from the norm. Typical test frequency is daily for most situations but the actual time can vary substantially. Therefore, many inferior films could be produced prior to running a control which may lead to an incorrect diagnosis or a need to repeat the exposure to the patient.

Faced with this chemical dilemma and the accepted American College of Radiography guidelines, the practitioner is forced into one of the following two situations. The first is a correct film measurement indicating the current chemistry may be correct but replenishment conditions are unknown. In this situation the practitioner typically continues operating with no knowledge of potential problems. The second situation occurs when the film measurements are not correct. Based on the standard guidelines an initial check of obvious problems such as temperature, and the like, is suggested. If the problem is not resolved the processing and replenishment chemicals are usually discarded and replaced at a substantial financial and time burden to the medical professional.

There is a long felt need in the art to provide means for improved quality control in film processing. There is a further need to provide a developer and replenisher therefore which purposefully contain ingredients that can be accurately and rapidly analyzed to determine the chemical activity of the solution. Described herein is a chemical development system wherein specific ingredients can be added and a potentiometric titration performed to insure proper levels of developer, replenisher, color chromophores and the like.

### Summary of the Invention:

It is an object of the present invention to provide an improved development method for silver halide films which can be easily monitored and can provide diagnostic information on the activity of the developer.

It is a further object to provide a developer solution, and replenisher therefore, which can provide diagnostic information on the activity of the developer and the replenisher from a single measurement.

It is a further object that the developer/replenisher solution can be monitored independent of the film thereby decreasing the effects of film, exposure and density measurements on the development conditions.

Yet another object is a diagnostic test method which can determine if the replenisher or developer is properly mixed and which can provide diagnostic information for correcting an improperly prepared solution.

A particular feature of the present invention is the ability to determine quantitative information rapidly and with minimal cost.

These and other advantages are provided in a method for converting a series of image-wise exposed silver halide photographic films to viewable images comprising the steps of:
(a) developing an image-wise exposed silver halide film in a first developer, with a pH of 9-12, wherein said first developer comprises:
   a developing agent in a first agent concentration, a first titratably distinct component in a first component concentration and a second titratably distinct component in a second component concentration,
   whereby said exposed silver halide is reduced to elemental silver and said first developer is depleted forming a depleted developer wherein said depleted developer comprises:
   said developing agent in a second agent concentration, said first titratably distinct component in a first depleted component concentration and said second titratably distinct component in said second depleted component concentration;
(b) removing unexposed silver halide from said photographic film with a fixing solution;
(c) titrating said depleted developer to determine a ratio of said first depleted component concentration and said second depleted component concentration;
(d) adding a replenishment solution to said depleted developer to form a replenished developer wherein said replenishment solution comprises:
   said developing agent, said first titratably distinct component and said second titratably component;
   wherein said replenished developer has a pH of 9-12 and comprises:
   said developing agent in said first agent concentration, said first titratably distinct component in said first component concentration and said second titratably distinct component in said second component concentration;
(e) repeating steps (a) through (d) for at least one additional imagewise exposed silver halide film.

In a particularly preferred embodiment the titratably distinct components are independently defined to have a Ksp between 10⁻⁶ and 10⁻²⁰. It is also preferred that the Ksp of the titratably distinct ions differ by at least 10⁻². Particularly preferred as titratably distinct components are bromide and chloride.

### Detailed Description of the Invention:

Chemical developers are specifically formulated to efficiently reduce image-wise exposed silver halide to elemental silver. The developer typically comprises a reducing agent, optional antifoggants, optional pH buffers, optional hardeners and optional stabilizers.

Each of at least two components of the replenisher further comprise compounds which are analytically distinct one from the other when the components are mixed. The term analytically distinct refers to compounds which are titratably distinct.

The term "titratably distinct" refers specifically to compounds which can be quantitatively distinguished in a single potentiometric titration with silver nitrate. The titration should be done at a pH of which is sufficient to insure that silver oxide formation does not occur. This pH is preferably no higher than 8.0.

Preferred titratably distinct components are anions which form silver salts and which do not adversely interfere with the photographic development or fix process. It is particularly important that the silver salts formed have sufficient solubility that premature precipitation does not alter the results. Preferred is a salt with a solubility product (Ksp) of 10⁻⁶ to 10⁻²⁰. Specifically preferred are combinations of anions which form silver salts with sufficient differences in solubility product to be quantitatively separatable in a potentiometric titration. The solubility products of the silver salts, measured as Ksp, are preferably different by at least 10⁻² using current titration abilities under ambient conditions. In a particularly preferred embodiment the bromide is one titrant and the other titrants are chosen accordingly. Chloride has been found to be particularly preferred as a second titrant due to the low cost, photographic inert properties, solubility and the like.

Preferred reducing agents (suitable for the developer and replenisher solutions) are 4-hydromxymethyl-1-phenyl-3-pyrazolidone, 1-phenyl-3-pyrazolidone, or a derivative thereof such as 4-methyl or 4,4-dimethyl-1-phenyl-3-pyrazolidone; hydroquinone or a derivative thereof such as chlorohydroquinone or bromohydroquinone; ascorbic acid; sugar-type derivatives of ascorbic acid; stereoisomers and diastereoisomers of ascorbic acid and their sugar-type derivatives; or salts of ascorbic acid or their derivatives ; and mixtures thereof.

Preferred reducing agents are hydroquinone, 4-hydroxymethyl-1-phenyl-3-pyrazolidone, 1-phenyl-3-pyrazolidone, ascorbic acid, d-erythroascorbic acid (i.e. erythorbic or isoascorbic acid), d-glucosascorbic acid, 6-deoxy-l-ascorbic acid, d-glucoascorbic acid, d-galactoascorbic acid, l-glucoascorbic acid and l-alloascorbic acid.

Exemplary salts of ascorbic acid, which are useful for the teachings herein, include alkali metal salts, such as the sodium and potassium salts thereof (e.g. sodium or potassium ascorbate and sodium or potassium erythorbate).

The unsubstituted compounds of this class of compounds may be represented by the formula: wherein X is an oxygen atom or imino group, R is any group which does not render the ascorbic acid water-insoluble and is a non-interfering group. Non-interfering is defined as not causing steric hindrance, is not chemically reactive with other portions of the molecule, is not a coordination group for the molecule, and is not more electropositive than a saturated hydrocarbon residue. R is preferably an aryl group, in particular an aryl group of 6-10 carbons, or a group of the formula R¹(CH₂)(CH₂)ₙ₋₁ wherein n is a positive integer from 1 to 4 and R1 is either a hydrogen atom or hydroxyl group when n is 2 to 4 and is hydroxyl when n is 1. Of these materials, ascorbic and erythorbic (iso-ascorbic) acid are preferred.

The developer may contain a multitude of conventional ingredients which serve functions well known in the art. Included are additional development agents, antifoggant agents, pH buffers, sequestering agents, swelling control agents and development accelerators. Materials which may be included in the processing solution, such as swelling control agents (i.e. gelatin hardening agents), aerial oxidation restrainers, sequestering agents, surfactants, dyes, well known in the art are exemplified in U.S. Pat. No. 3,545,971 and Photographic Processing Chemistry, L.F.A. Mason, 1966, page 149 et seq.

Other reducing agents which may be used are organic agents such as catechols, aminophenols, phenylenediamines, tetrahydroquinolines, bis(pyridone)amines, cylcoalkenones, pyrimidines, reductones and coumarins. Inorganic development agents may also be mentioned to include metals having at least two distinct valence states and are capable of reducing ionic silver to metallic silver. Such metals include iron, titanium, vanadium and chromium and it is preferable to employ the metals with organic compounds such as polycarboxylic acids or aminopolycarboxylic acids.

The organic antifoggant may be any organic antifoggant or film speed restrainer. Such organic antifoggants are commonly employed in X-ray developer baths and include compounds such as benzimidazole, benzotriazole, benzothiazole, indazole, tetrazole, imidazole, mercaptotetrazole and thiazole group, as well as anthraquinone sulfonic acid salts. Two or more organic antifoggants may be used. It is preferred to use a mixture or two antifoggants such as 5-nitroindazole and benzotriazole. Sodium or potassium bromides are also suitable.

Exemplary sequestering agents include but are not limited to aminopolycarboxylic acid compounds, ethylenediaminetetraacetic acid, and sodium salts thereof, diethylenetriaminepentaacetic acid, diaminopropanoltetraacetic acid, gluconic acid and its salts, hepto and borogluconates, citric acid and its salts.

Exemplary swell control agents are dialdehydes or diketones particularly glyoxal, or homologous of glyoxal in which the two aldehyde groups are seperated by a chain of 2 or 3 carbon atoms. Preferred is glutaraldehyde. Other compounds which may be mentioned include diacetyl, acetyl benzoyl and dichlorodiacetyl.

It is imperative that a developer pH of approximately 9-12 be maintained. More preferred is a developer pH of 9.7-10.6 and most preferred is a developer pH of 10.0±0.3. Any alkaline material may be used to provide the required pH, such as sodium or potassium hydroxide, sodium or potassium carbonate. The buffer system may be any convenient system, e.g., the borate and carbonate buffers conventionally used in X-ray developer baths are quite suitable.

The replenisher solution is ideally formulated such that addition to the developer restores the chemical composition of the developer to optimal composition under steady state conditions. It is typically preferred that the replenisher be substantially identical to the developer with the exception of the titratably distinct additives described herein.

The term Ksp is standard in the art and refers specifically to the solubility product constant. The solubility constant can be defined as the product of the concentration of the ions of a substance in a saturated solution of the substance. For purposes of this invention the solubility product in water, at ambient temperatures, is a sufficiently close approximation to the solubility product in processing chemicals.

If more than two replenisher components are to be monitored then multiple salts can be used with the proviso that at least two meet the criteria described above. Another embodiment includes the use of two salts with at least one salt used in multiple samples. In this embodiment the concentration of salt in the component would be such that when all of the components are added the deviations from ideal concentration would be detectable as shown in Example 1.

The preferred developer composition and replenisher therefore comprises, per liter: 0.5 to 5.0 g of 1-phenyl-3-pyrazolidone or a derivative thereof; 15 to 35 g of hydroquinone, or a derivative thereof; 0 to 10 g of bromide ion; 0.01 to 6.0 mmoles of an organic antifoggant; 1.0 to 30.0 g of a titratably distinct ion and 0 to 30 g of a different titratably distinct ion. When bromide ion is present it is preferred that the second titratably distinct ion is chloride.

Another preferred developer composition and replenisher comprises, per liter, 15.0 to 75.0 g of ascorbic acid; 0.5 to 5.0 g of 3-pyrazolidone or a suitable derivative thereof; 2 to 20 grams of sulfite; 15 to 30 grams of carbonate; 0 to 10 g of bromide ion; 0.01 to 6.0 mmoles of an organic antifoggant; 1.0 to 30.0 g of a titratably distinct ion and 0 to 30.0 g of a different titratably distinct ion.

One embodiment, in accordance with the teachings herein, is the inclusion of one titratably distinct salt with the reducing agent and one titratably distinct salt with a second replenisher component. Particularly preferred is a composition with one titratably distinct salt added in an amount which is directly proportional to the reducing agent, and the second titratably distinct salt added in an amount which is directly proportional to the glutaraldehyde bisulfite.

It has long been the practice in the art to provide the customer with concentrated solutions which are then mixed prior to use or placed in an automatic mixer as detailed in U.S. Patent 4,741,991. In this embodiment it is particularly preferred that titratably distinct ions be included in each solution. A potentiometric titration can then be used to insure that mixing is accurate prior to replenishing the working developer.

A range of bromide ion can be used successfully in this invention. It is preferred that one of the titratably distinct ions be KBr in an amount equal to 1 to 10 g/liter. NaBr may also be employed. Optimum amounts depend on replenishment rate and specific formula.

These essential ingredients, when dissolved in water at the concentrations set forth above, enable the photographic solution to be used in the invention to function as a developer bath and a shelf-stable replenisher.

Conventionally, all of the ingredients of the developer are prepared in concentrated form in water. Separate portions of the concentrates are furnished users so that interaction between ingredients is lessened while in this concentrated state. Then, the user makes up the developer solution by measuring various amounts from each part and mixing with water to achieve the desired solution. The pH is then adjusted, e.g., to 10.0±0.3, and the solution charged to the processing tank, e.g., of the type described in U.S. Pat. No. 3,545,971, such as an "X-Omat Processor", in the amount required by the system. Development time is determined empirically or by the processor. Replenishment will be carried out at a rate per unit area of exposed film without change in sensitometric properties of the film, and will be determined empirically, as well known. As a guide, when using an X-Omat Processor to process X-ray film, a suitable replenishment rate will be 50-70 ml per 0.155 m² (240 square inches) of film (40% exposed) for development to normal radiographic density, using the processing solution of the invention as properly prepared.

Substantially all processors have some type of a standby replenishment mode. There are a lot of differences based on the manufacturer but the concept is usually similar. The standby mode typically works as follows: if no film is passed in a given time, the processor goes into a standby mode which deactivates the drive train and dryer and reduces the water supply. After a given time, it comes back on for several minutes and then shuts off again. After a specified number of cycles, it replenishes a predetermined amount.

Potentiometric titrations are well known in the art as exemplified in Instrumental Analysis, Bauer, Christian, O'Reilly, Alyyn and Bacon, 1979, Chapter 2.

The following example 2 is intended to further illustrate and demonstrate the teachings of this invention.

### EXAMPLE 1

An example of the use of three components with two salts is as follows:
Solution 1 would contain salt A at a level sufficient to equal 4 g/l in the final mixture, Solution 2 would contain salt B at a level sufficient to equal 4 g/l in the final mixture, Solution 3 would contain salt A at a level sufficient to equal 1 g/l and salt B at a level sufficient to equal 1 g/l in the final mixture. A properly prepared replenisher would be expected to contain 5 g/l of both salt A and salt B. If Solution 1 is added incorrectly then salt A will deviate from 5 g/l but salt B will be correct and so forth.

### EXAMPLE 2

Three stock solutions were prepared in accordance with U.S. Patent 4,741,991. Sodium chloride was added to Solution C to demonstrate the utility of the current invention. For this example diagnostic analysis is restricted to two solutions only to facilitate understanding of the inventive concept. Expansion to more solutions could be accomplished as detailed in Example 1.

| Ingredients | Amt (g) |
|---|---|
| Solution A | |
| Dist. Water | ca. 3785 |
| EDTA | 75 |
| Sodium Bisulfite | 1428 |
| Hydroquinone | 946 |
| KOH (45% aq.) | 3075 |
| KOH (solid) | 1383 |
| Sodium Bicarbonate | 315 |
| KBr | 113 |
| Dist. Water to | 9.46 liters |

| Solution B | |
|---|---|
| Triethylene Glycol | 402 |
| Acetic Acid | 270 |
| Phenidone | 60 |
| 5-nitroindazole | 6 |
| Benzotriazole | 8 |
| Dist. Water to | 1 liter |

| Solution C | |
|---|---|
| Water | 500 |
| Glutaraldehyde (50% aq.) | 267 |
| Sodium Bisulfite (anhydr.) | 106 |
| Sodium Chloride | 67.56 |
| Dist. Water to | 1 liter |

Specific mixtures of these ingredients were prepared as replenishment solutions which are chosen to simulate actual operating conditions commonly encountered in a processor. This mixture is intended for use with a replenisher which has a constant bromide level of 3.0 g/l, as sodium salt, and a pH of 10.0 ± 0.3. The specific solutions are detailed below.

| R1 - representing a properly prepared replenisher solution | |
|---|---|
| Water | 700 ml |
| Solution A | 250 ml |
| Solution B | 25 ml |
| Solution C | 25 ml |

| R2 - representing a replenisher which is 10% overdiluted | |
|---|---|
| Solution R1 | 250 ml |
| Water | 25 ml |

| R3 - representing a replenisher which is 15% overdiluted | |
|---|---|
| Solution R1 | 250 ml |
| Water | 37.5 ml |

| R4 - representing replenisher with proper dilution but 10% shortage of | |
|---|---|
| Solution A | |
| Water | 725 ml |
| Solution A | 225 ml |
| Solution B | 25 ml |
| Solution C | 25 ml |

| R5 - representing replenisher with proper dilution but 10% shortage of | |
|---|---|
| Solution C | |
| Water | 702.5 ml |
| Solution A | 250 ml |
| Solution B | 25 ml |
| Solution C | 22.5 ml |

| R6 - representing a solution which is properly mixed but underdiluted by 10% | |
|---|---|
| Water | 600 ml |
| Solution A | 250 ml |
| Solution B | 25 ml |
| Solution C | 25 ml |

Standard pH and specific gravity measurements were taken and the halides were titrated using the following procedure. A 10 ml sample was taken from each solution. The sample was diluted to 120 ml with 0.1 N sulfuric acid. The samples were then titrated for bromide ion and chloride ion, in triplicate, using the two endpoint potentiometric method on a Brinkman Model 702 automatic titrator using a silver billet electrode. The halide ion concentration was reported as a sodium salt. The pH was measured with a Fisher Accumet 915 pH meter equipped with a combination glass electrode as known in the art. Specific gravity was determined by weighing 10 ml samples. The results are listed in Table 1.

**TABLE 1**

| Replenisher | pH | SG | Br | Cl |
|---|---|---|---|---|
| R1 | 10.10 | 1.81 | 3.05 | 1.69 |
| R2 | 10.10 | 1.72 | 2.81 | 1.51 |
| R3 | 10.11 | 1.71 | 2.68 | 1.46 |
| R4 | 10.02 | 1.72 | 2.75 | 1.69 |
| R5 | 10.13 | 1.79 | 3.02 | 1.55 |
| R6 | 10.16 | 1.90 | 3.42 | 2.00 |
| SG is specific gravity in g/l, Br and Cl are both in g/l as sodium salt. | | | | |

Expected values for pH are 10.1 ± 0.1 which suggest that all of these solutions are within the normal operating range and are therefore considered acceptable for use even though they were purposely prepared incorrectly.

Except for the sodium chloride, the replenisher illustrated is substantially identical to that described in U.S. Pat. No. 4,741,991. This replenisher is intended to be used with a developer which has a steady state bromide level of 6.0 to 7.0 g/l as the sodium salt. As expected the development reaction would cause the bromide ion level to increase as film is developed in accordance with Equation 1. The combined teachings of U.S. Pat. No. 4,741,991 and U.S. Pat. No. 3,970,457 would suggest that the replenisher is added in an amount sufficient to return the bromide ion level to the predetermined level. Addition of a replenisher with a bromide ion level of 3.0 g/l as the sodium salt would effectively dilute the bromide ion concentration thereby counteracting the effect of use as described herein. Using only a bromide ion titration on the developer, and a replenisher with an expected bromide level of 3.0 g/l as the sodium salt, the replenishment for each sample would yield different results. The developer replenished with R2, R3 or R4 would be under replenished since not as much solution would be required to lower the bromide ion concentration to a predetermined level. Even though the bromide ion level would be corrected the HOC₆H₄OSO₃Na would not be replaced with unreacted hydroquinone and sulfite. Therefore, a continuous bromide ion titration on the developer would not offer any diagnostic information. The developer replenished with R5 would have the proper amount of hydroquinone added but would be deficient of sulfite and glutaraldehyde. The deficiency in sulfite and glutaraldehyde would be completely transparant from the bromide ion titration alone. The developer replenished with R6 would also be incorrectly replenished since the bromide ion concentration added to the developer would be higher, on a volume basis, than expected.

Depending on the film used a processor upset may be detected for each of R2 through R6 with no diagnostic information available based on the bromide ion titration alone.

Using identical solutions and analyzing both the bromide and chloride ion solutions, in accordance with this invention, provides an immediate indication of improper mixing. The four distinct possibilities which exist for the replenisher in this example are:
1) both halide ions are on aim (i.e. R1)
2) both halides are either above or below aim (i.e. R2, R3, R6)
3) one halide ion is high and the other is low
4) one halide ion is off aim or missing (i.e. R4, R5).

A titration of the developer replenished with R1 would have the predetermined level of bromide ion and chloride ion. A titration of the developer replenished with a set amount of R2 or R3 would have a bromide ion level which is lower than the predetermined level and a chloride ion level which is below the predetermined level. A developer replenished with a set amount of R4 would have a bromide ion level which is lower than the predetermined level and a chloride ion level which is at the predetermined level. A developer replenished with a set amount of R5 would have a bromide ion level which is at the predetermined level and a chloride ion level which is low. A developer replenished with a set amount of R6 would have a bromide and chloride level which is above the predetermined levels. In all cases the incorrect solution could be immediately corrected by changing replenishment amount or adding one component of replenisher.

These diagnostics could then be used to properly adjust the solutions and/or the replenishment rate to achieve the appropriate results. Based on these examples the replenishment rate could be increased by the appropriate factor when samples such as R2 and R3 are observed. R4 and R5 could be remixed with additional ingredients to achieve the proper balance of bromide ion to chloride ion and the replenishment adjusted accordingly. R6 could be diluted to the appropriate level and the problem alleviated. In each of these examples the current practice of replacing the entire chemical charge and remixing could be avoided since the mixture could be corrected.

Furthermore, once the above mentioned corrections are made a retest can be used to certify that the replenishment, and development are correct without the use of film.

## Claims

1. A method for converting a series of image-wise exposed silver halide photographic films to viewable images comprising the steps of:
(a) developing an image-wise exposed silver halide film in a first developer, with a pH of 9-12, wherein said first developer comprises:
a developing agent in a first agent concentration, a first titratably distinct component in a first component concentration and a second titratably distinct component in a second component concentration,
whereby said exposed silver halide is reduced to elemental silver and said first developer is depleted forming a depleted developer wherein said depleted developer comprises:
said developing agent in a second agent concentration, said first titratably distinct component in a first depleted component concentration and said second titratably distinct component in said second depleted component concentration;
(b) removing unexposed silver halide from said photographic film with a fixing solution;
(c) titrating said depleted developer to determine a ratio of said first depleted component concentration and said second depleted component concentration;
(d) adding a replenishment solution to said depleted developer to form a replenished developer wherein said replenishment solution comprises:
said developing agent, said first titratably distinct component and said second titratably component;
wherein said replenished developer has a pH of 9-12 and comprises:
said developing agent in said first agent concentration, said first titratably distinct component in said first component concentration and said second titratably distinct component in said second component concentration;
(e) repeating steps (a) through (d) for at least one additional imagewise exposed silver halide film.

2. The method recited in Claim 1 wherein said first titratably distinct component and said second titratably distinct component independently form silver salts with a Ksp value between 10^{- 6} and 10^{- 20}.

3. The method recited in Claim 1 wherein said first titratably distinct component and said second titratably distinct component have a Ksp value which differs by at least 10^{- 2}.

4. The method recited in Claim 1 wherein said first titratably distinct component is bromide.

5. The method recited in Claim 1 wherein said second titratably distinct component is chloride.

6. The method recited in Claim 1 wherein said developing agent is chosen from a set consisting of 4-hydroxymethyl-1-phenyl-3-pyrazolidone, 1-phenyl-3-pyrazolidone, 4-methyl-1-phenyl-3-pyrazolidone; 4,4-methyl-1-phenyl-3-pyrazolidone; hydroquinone, chlorohydroquinone and bromohydroquinone.

7. The method recited in Claim 1 wherein said replenishment solution comprises, per liter, 0.5 to 5.0 g of 1-phenyl-3-pyrazoline; 15 to 35 g of hydroquinone; 0 to 10 g of bromide; 0.01 to 6.0 mmoles of an organic antifoggant; 1.0 to 30.0 g of said first titratably distinct ion and 0.0 to 30 g of said second titratably distinct ion, if said bromide is present in an amount equal to 0 g per liter said second titratably distinct ion can not be present in an amount equal to 0.0 g per liter.

8. The method recited in Claim 1 wherein said developing agent comprises at least one compound chosen from the set consisting of ascorbic acid, sugar derivatives of ascorbic acid, stereoisomers of ascorbic acid, diastereoisomers of ascorbic acid, salts of ascorbic acid and mixtures thereof.

9. The method recited in Claim 8 wherein said developing agent comprises at least one compound chosen from the set consisting of ascorbic acid, d-erythro-ascorbic acid (i.e. erythorbic or isoascorbic acid), d-glucosascorbic acid, 6-deoxy-l-ascorbic acid, d-glucoascorbic acid, d-galactoascorbic acid, l-guloascorbic acid and l-alloascorbic acid.

10. The method recited in Claim 1 wherein said replenishment solution comprises, per liter, 15.0 to 75.0 g of ascorbic acid; 0.5 to 5.0 g of 3-pyrazolidone or a suitable derivative thereof; 2 to 20 grams of sulfite; 15 to 30 grams of carbonate; 0 to 10 g of bromide ion; 0.01 to 6.0 mmoles of an organic antifoggant; 1.0 to 30.0 g of said first titratably distinct ion and 0 to 30.0 g of said second titratably distinct ion, if said bromide is present in an amount equal to 0 g per liter said second titratably distinct ion can not be present in an amount equal to 0.0 g per liter.

11. The method recited in Claim 8 wherein said development agent comprises: wherein:
X is an oxygen atom or imino group;
R is an aryl group or a group of the formula R¹(CH₂)(CH₂)ₙ₋₁ wherein n is a positive integer from 1 to 4 and R¹ is either a hydrogen atom or hydroxyl group when n is 2 to 4 and is hydroxyl when n is 1.

12. The method recited in Claim 1 wherein said development agent is wherein:
X is an oxygen atom or imino group; and
R is any group which does not render the ascorbic acid water-insoluble and is a non-interfering group.

## Patentansprüche

1. Verfahren zur Umwandlung einer Serie von bildmäßig belichteten fotografischen Silberhalogenidfolien in beobachtbare Bilder, mit folgenden Stufen :
(a) die Entwicklung einer bildmäßig belichteten Silberhalogenid-folie in einem ersten Entwickler mit einem pH zwischen 9 und 12, wobei dieser erste Entwickler die nachstehenden Ingredienzien enthält :
eine Entwicklersubstanz in einer ersten Substanzkonzentration, eine erste titrierbar unterschiedliche Komponente in einer ersten Komponentenkonzentration und eine zweite titrierbar unterschiedliche Komponente in einer zweiten Komponentenkonzentration,
wobei das belichtete Silberhalogenid zu elementarem Silber reduziert wird und sich der erste Entwickler abreichert, wodurch ein abgereicherter Entwickler erhalten wird, der die nachstehenden Ingredienzien enthält :
die Entwicklersubstanz in einer zweiten Substanzkonzentration, die erste titrierbar unterschiedliche Komponente in einer ersten abgereicherten Komponentenkonzentration und die zweite titrierbar unterschiedliche Komponente in einer zweiten abgereicherten Komponentenkonzentration,
(b) die Entfernung des unbelichteten Silberhalogenids von der fotografischen Folie mit Hilfe einer Fixierlösung,
(c) die Titrierung des abgereicherten Entwicklers zur Ermittlung des Verhältnisses der ersten abgereicherten Komponentenkonzentration zur zweiten abgereicherten Komponentenkonzentration,
(d) die Zugabe einer Nachfüllösung im abgereicherten Entwickler, wodurch ein nachgefüllter Entwickler erhalten wird, der die nachstehenden Ingredienzien enthält :
die Entwicklersubstanz, die erste titrierbar unterschiedliche Komponente und die zweite titrierbar unterschiedliche Komponente,
wobei der nachgefüllte Entwickler einen pH zwischen 9 und 12 aufweist und folgende Ingredienzien enthält :
die Entwicklersubstanz in der ersten Substanzkonzentration, die erste titrierbar unterschiedliche Komponente in der ersten Komponentenkonzentration und die zweite titrierbar unterschiedliche Komponente in der zweiten Komponentenkonzentration,
(e) die Wiederholung der Stufen (a) bis (d) für wenigstens eine zusätzliche bildmäßig belichtete Silberhalogenidfolie.

2. Verfahren nach Anspruch 1, dadurch gekennzeichnet, daß die erste titrierbar unterschiedliche Komponente und die zweite titrierbar unterschiedliche Komponente unabhängig voneinander Silbersalze mit einem Ksp-Wert zwischen 10⁻⁶ und 10⁻²⁰ bilden.

3. Verfahren nach Anspruch 1, dadurch gekennzeichnet, daß der Ksp-Wert der ersten titrierbar unterschiedlichen Komponente und der Ksp-Wert der zweiten titrierbar unterschiedlichen Komponente um wenigstens 10⁻² auseinander liegen.

4. Verfahren nach Anspruch 1, dadurch gekennzeichnet, daß die erste titrierbar unterschiedliche Komponente Bromid ist.

5. Verfahren nach Anspruch 1, dadurch gekennzeichnet, daß die zweite titrierbar unterschiedliche Komponente Chlorid ist.

6. Verfahren nach Anspruch 1, dadurch gekennzeichnet, daß die Entwicklersubstanz 4-Hydroxymethyl-1-phenyl-3-pyrazolidon, 1-Phenyl-3-pyrazolidon, 4-Methyl-1-phenyl-3-pyrazolidon, 4,4-Methyl-1-phenyl-3-pyrazolidon, Hydrochinon, Chlorhydrochinon oder Bromhydrochinon ist.

7. Verfahren nach Anspruch 1, dadurch gekennzeichnet, daß die Nachfüllösung pro Liter zwischen 0,5 und 5,0 g 1-Phenyl-3-pyrazolin, zwischen 15 und 35 g Hydrochinon, zwischen 0 und 10 g Bromid, zwischen 0,01 und 6,0 Mmol eines organischen Schleierschutzmittels, zwischen 1,0 und 30,0 g des ersten titrierbar unterschiedlichen Tons und zwischen 0,0 und 30 g des zweiten titrierbar unterschiedlichen Tons enthält, wobei das zweite titrierbar unterschiedliche Ion nicht in einer Menge von 0,0 g pro Liter enthalten sein kann, wenn das Bromid in einer Menge von 0 g pro Liter enthalten ist.

8. Verfahren nach Anspruch 1, dadurch gekennzeichnet, daß die Entwicklersubstanz wenigstens eine Verbindung aus der Gruppe bestehend aus Ascorbinsäure, Zucker-Derivaten von Ascorbinsäure, Stereoisomeren von Ascorbinsäure, Diastereoisomeren von Ascorbinsäure, Salzen von Ascorbinsäure und Gemischen derselben enthält.

9. Verfahren nach Anspruch 8, dadurch gekennzeichnet, daß die Entwicklersubstanz wenigstens eine Verbindung aus der Gruppe bestehend aus Ascorbinsäure, d-Erythroascorbinsäure (d.h. Erythorbinsäure oder Isoascorbinsäure), d-Glucosascorbinsäure, 6-Deoxy-l-ascorbinsäure, d-Glucoascorbinsäure, d-Galacto-ascorbinsäure, l-Guloascorbinsäure und l-Alloascorbinsäure enthält.

10. Verfahren nach Anspruch 1, dadurch gekennzeichnet, daß die Nachfüllösung pro Liter zwischen 15,0 und 75,0 g Ascorbinsäure, zwischen 0,5 und 5,0 g 3-Pyrazolidon oder eines geeigneten Derivats davon, zwischen 2 und 20 g Sulfit, zwischen 15 und 30 g Carbonat, zwischen 0 und 10 g Bromid, zwischen 0,01 und 6,0 Mmol eines organischen Schleierschutzmittels, zwischen 1,0 und 30,0 g des ersten titrierbar unterschiedlichen Ions und zwischen 0 und 30 g des zweiten titrierbar unterschiedlichen Ions enthält, wobei das zweite titrierbar unterschiedliche Ion nicht in einer Menge von 0,0 g pro Liter enthalten sein kann, wenn das Bromid in einer Menge von 0 g pro Liter enthalten ist.

11. Verfahren nach Anspruch 8, dadurch gekennzeichnet, daß die Entwicklersubstanz enthält,
wobei bedeuten :
X ein Sauerstoffatom oder eine Iminogruppe,
R eine Arylgruppe oder eine Gruppe der Formel R¹(CH₂)(CH₂)ₙ₋₁, wobei n eine positive ganze Zahl zwischen 1 und 4 und R¹ entweder ein Wasserstoffatom oder eine Hydroxylgruppe bedeutet, falls n zwischen 2 und 4 liegt, und eine Hydroxylgruppe bedeutet, falls n 1 ist.

12. Verfahren nach Anspruch 1, dadurch gekennzeichnet, daß die Entwicklersubstanz ist,
wobei X ein Sauerstoffatom oder eine Iminogruppe bedeutet und R irgendwelche Gruppe bedeuten kann, die die Ascorbinsäure nicht wasserunlöslich zu machen vermag und keine störende Gruppe ist.

## Revendications

1. Procédé pour transformer une série de films photographiques à l'halogénure d'argent exposés en forme d'image en images visibles, comprenant les étapes consistant à:
(a) développer un film à l'halogénure d'argent exposé en forme d'image dans un premier révélateur possédant un pH de 9-12, dans lequel ledit premier révélateur comprend:
un agent développateur dans une première concentration d'agent, un premier composant que l'on peut distinguer par titrage dans une première concentration de composant et un second composant que l'on peut distinguer par titrage dans une seconde concentration de composant,
par lequel, ledit halogénure d'argent exposé est réduit en argent élémentaire et ledit premier révélateur est épuisé pour former un révélateur à l'état épuisé dans lequel ledit révélateur à l'état épuisé comprend:
ledit agent développateur dans une seconde concentration d'agent, ledit premier composant que l'on peut distinguer par titrage dans une première concentration de composant à l'état épuisé et ledit second composant que l'on peut distinguer par titrage dans ladite seconde concentration de composant à l'état épuisé;
(b) éliminer l'halogénure d'argent non exposé dudit film photographique avec une solution de fixage;
(c) titrer ledit révélateur à l'état épuisé pour déterminer un rapport de ladite première concentration de composant à l'état épuisé et de ladite seconde concentration de composant à l'état épuisé;
(d) ajouter une solution de régénération audit révélateur à l'état épuisé pour former un révélateur régénéré dans lequel ladite solution de régénération comprend:
ledit agent développateur, ledit premier composant que l'on peut distinguer par titrage et ledit second composant que l'on peut distinguer par titrage;
dans lequel ledit révélateur régénéré possède un pH de 9-12 et comprend:
ledit agent développateur dans ladite première concentration d'agent, ledit premier composant que l'on peut distinguer par titrage dans ladite première concentration de composant et ledit second composant que l'on peut distinguer par titrage dans ladite seconde concentration de composant;
(e) répéter les étapes (a) à (d) pour au moins un film supplémentaire à l'halogénure d'argent exposé en forme d'image.

2. Procédé selon la revendication 1, dans lequel ledit premier composant que l'on peut distinguer par titrage et ledit second composant que l'on peut distinguer par titrage forment, indépendamment l'un de l'autre, des sels d'argent possédant une valeur Ksp entre 10⁻⁶ et 10⁻²⁰.

3. Procédé selon la revendication 1, dans lequel ledit premier composant que l'on peut distinguer par titrage et ledit second composant que l'on peut distinguer par titrage possèdent des valeurs Ksp dont la différence s'élève à au moins 10⁻².

4. Procédé selon la revendication 1, dans lequel ledit premier composant que l'on peut distinguer par titrage est un bromure.

5. Procédé selon la revendication 1, dans lequel ledit second composant que l'on peut distinguer par titrage est un chlorure.

6. Procédé selon la revendication 1, dans lequel ledit agent développateur est choisi parmi le groupe constitué par la 4-hydroxyméthyl-1-phényl-3-pyrazolidone, la 1-phényl-3-pyrazolidone, la 4-méthyl-1-phényl-3-pyrazolidone, la 4,4-méthyl-1-phényl-3-pyrazolidone, l'hydroquinone, la chlorohydroquinone et la bromohydroquinone.

7. Procédé selon la revendication 1, dans lequel ladite solution de régénération comprend, par litre, de 0,5 à 5,0 g de la 1-phényl-3-pyrazolidone; de 15 à 35 g d'hydroquinone; de 0 à 10 g de bromure; de 0,01 à 6,0 mmoles d'un agent antivoile organique; de 1,0 à 30,0 g dudit premier ion que l'on peut distinguer par titrage et de 0,0 à 30 g dudit second ion que l'on peut distinguer par titrage; lorsque ledit bromure est présent en une quantité égale à 0 g par litre, ledit second ion que l'on peut distinguer par titrage ne peut être présent en une quantité égale à 0,0 g par litre.

8. Procédé selon la revendication 1, dans lequel ledit agent développateur comprend au moins un composé choisi parmi le groupe constitué par l'acide ascorbique, des dérivés de sucre de l'acide ascorbique, des stéréo-isomères de l'acide ascorbique, des diastéréo-isomères de l'acide ascorbique, des sels de l'acide ascorbique et leurs mélanges.

9. Procédé selon la revendication 8, dans lequel ledit agent développateur comprend au moins un composé choisi parmi le groupe constitué par l'acide ascorbique, l'acide d-érythro-ascorbique (c'est-à-dire l'acide érythorbique ou l'acide isoascorbique), l'acide d-glucosascorbique, l'acide 6-désoxy-1-ascorbique, l'acide d-glucosascorbique, l'acide d-galactoascorbique, l'acide l-guloascorbique et l'acide l-allo-ascorbique.

10. Procédé selon la revendication 1, dans lequel ladite solution de régénération comprend, par litre, de 15,0 à 75,0 g d'acide ascorbique; de 0,5 à 5,0 g de 3-pyrazolidone ou d'un de ses dérivés; de 2 à 20 g de sulfite; de 15 à 30 g de carbonate; de 0 à 10 g d'ion bromure; de 0,01 à 6,0 moles d'un agent antivoile organique; de 1,0 à 30,0 g dudit premier ion que l'on peut distinguer par titrage; et de 0 à 30,0 g dudit second ion que l'on peut distinguer par titrage; lorsque ledit bromure est présent en une quantité égale à 0 g par litre, ledit second ion que l'on peut distinguer par titrage ne peut être présent en une quantité égale à 0,0 g par litre.

11. Procédé selon la revendication 8, dans lequel ledit agent développateur comprend: formule dans laquelle:
X représente un atome d'oxygène ou un groupe imino;
R représente un groupe aryle ou un groupe répondant à la formule R¹(CH₂)(CH₂)ₙ₋₁ où n représente un entier positif de 1 à 4 et R¹ représente, soit un atome d'hydrogène, soit un groupe hydroxyle lorsque n est égal à 2-4 et représente un groupe hydroxyle lorsque n est égal à 1.

12. Procédé selon la revendication 1, dans lequel ledit agent développateur et répond à la formule: dans laquelle:
X représente un atome d'oxygène ou un groupe imino; et
R représente n'importe quel groupe qui ne rend pas l'acide ascorbique insoluble dans l'eau et représente un groupe qui n'interfère pas.
